

Jan. 27, 1948.

J. B. JOHNSON

2,434,930

METHOD AND APPARATUS FOR IONIC DISCHARGE COATING

Filed Dec. 1, 1944

2 Sheets-Sheet 1

FIG. 1



FIG. 2



INVENTOR  
J.B.JOHNSON  
BY  
Hugh S. Wertz  
ATTORNEY

Jan. 27, 1948.

J. B. JOHNSON

2,434,930

METHOD AND APPARATUS FOR IONIC DISCHARGE COATING

Filed Dec. 1, 1944

2 Sheets-Sheet 2



INVENTOR  
J. B. JOHNSON  
BY *Hugh S. Wertz*  
ATTORNEY

## UNITED STATES PATENT OFFICE

2,434,930

METHOD AND APPARATUS FOR IONIC  
DISCHARGE COATINGJohn B. Johnson, Maplewood, N. J., assignor to  
Bell Telephone Laboratories, Incorporated,  
New York, N. Y., a corporation of New York

Application December 1, 1944, Serial No. 566,062

12 Claims. (Cl. 117—33.2)

1

2

This invention relates to method and apparatus for ionic discharge coating and more specifically to methods of and means for generating positive ion beams and for utilizing said beams, for example, in the formation of targets for electron beams in electron camera tubes.

One well-known type of electron camera tube is called the "iconoscope." In the usual form of this tube there is provided a mosaic target comprising a metal backing or signal plate, an insulating layer on the signal plate, and a discontinuous layer of photosensitized metallic globules or particles on the insulating layer. Radiations from an object are applied to this target and it is scanned with a beam of electrons to produce a signal current in a resistor which is connected to the signal plate. In a well-known method of making mosaic targets, the insulating layer, which usually is of mica or glass, is coated with a metallic layer of silver and by a heating process the silver is broken up into discontinuous particles which are oxidized and sensitized with caesium to form caesium-oxide-silver globules. In screens made by this process, the particles are of irregular shape and distribution, thus leading to non-uniformity of photosensitivity over the surface of the mosaic. This invention in one of its primary aspects relates to mosaic targets in which this non-uniformity is avoided or greatly reduced.

It is an object of this invention to provide novel methods of and means for making mosaic targets for electrons, the particles of the mosaic being of substantially uniform shape, size and distribution.

In a copending application of the same inventor, Serial No. 484,966, filed April 29, 1943, there are described various methods and means of utilizing beams of positive ions of metallic material in the formation of mosaic targets. The ions may be of a metal which is photosensitive, such as an alkali or alkaline earth metal, or they may be of a metal which is not appreciably photosensitive. In this latter instance, the metallic spots formed by the method described in this copending application are photosensitized as in the usual iconoscope target technique.

In accordance with the present invention, a reducing positive ion beam as, for example, a beam of positively charged hydrogen ions, is produced by ion-optical means and utilized to scan a metallic oxide or other suitable non-conducting layer to produce "islands" of metal in a "sea" of insulation. Oxides of aluminum or beryllium, for example, are suitable for this purpose. In general, any of the oxides of the solid metals of group II of the periodic table according to Mendeleeff can be used. The "islands" of metal are then photosensitized as in the usual iconoscope technique.

More specifically, in accordance with an exemplary form of the invention, a hydrogen positive ion beam is generated in a side tube connected to the camera tube. This side tube comprises an evacuated container enclosing a first electrode member and one or more additional electrode members. Hydrogen is introduced into the side tube and a positive ion discharge is set up within the container which discharge is formed into a beam of ions by placing the additional electrode members at appropriate negative potentials with respect to the first electrode member to focus the positive ions into a beam. This beam of hydrogen positive ions is directed into the tube containing the target to be formed and there utilized as described above.

The target can have as a backing an insulating plate such as mica, backed by a metallic electrode. The aluminum or other oxide coating can be formed by first plating a coat of aluminum on the mica and then oxidizing this coating by any well-known means. This oxide coating then has metal islands formed in it by the reducing action of the hydrogen ion beam. An alternate way of forming the target is to use a plate of aluminum (or a solid metal from group II) or a plate of other metal on which aluminum is plated, oxidizing this aluminum to a predetermined depth, and then producing the islands of metal of a lesser depth than the oxide so that the oxide layer insulates under the islands as well as around them.

In the presence of normal hydrogen, the metal oxides are reduced extremely slowly, but under the impingement of ionized hydrogen the reduction is accelerated if at the same time the water vapor which is the decomposition product is pumped away thoroughly. The process therefore contemplates the circulation of very dry hydrogen at low pressure through the tube during the reduction operation.

In a specific method of operation, the hydrogen ion beam is caused to scan (by electromagnetic or electrostatic means) every elemental area of the desired portion of the non-conducting reducible material on which the discontinuous photosensitive elements are to be formed. The beam is varied in intensity during scanning so as to produce a regular pattern. One way of doing this is to cut off the beam in alternate spot scanning periods and also to cut off the beam during alternate line scanning periods so that a regular pattern of dots or squares interspersed with insulating areas is produced. The size of each dot or square is preferably made smaller than a picture element as determined by the size of the electron beam in the electron camera tube although it can be as large as the picture element or even larger. It will take many seconds or even minutes to scan the complete target in order

to produce the spot of metal of the required thickness.

By an alternative method, the target can be formed by repeated scanning, that is, a tiny increment of metal is formed by the reduction process on each elemental area and this increment is increased by other increments on succeeding scannings until the complete dot structure is built up.

As the photosensitized target loses its sensitivity when exposed to air, the gun system for the electron beam is preferably mounted in the tube before the ionizing process. The gun system for the positive ion beam is mounted in a side tube which is joined to the main tube. Hydrogen is admitted into the side tube and a positive ion beam is formed and the ion beam is caused to scan the target. After portions of the target are reduced by the ion beam, the connection between the main tube and the side tube is sealed off, the main tube is pumped, the target subjected to any heat treatments and partial oxidation which are necessary, and the tube sealed off.

The invention will be more readily understood by referring to the following description taken in connection with the accompanying drawings forming a part thereof in which:

Fig. 1 is a schematic diagram to illustrate a process, in accordance with this invention, of making a target for an electron camera tube by means of a reducing ion beam;

Fig. 2 is an enlarged view of a portion of the target for the ion beam; and

Fig. 3 shows a modification of the arrangement shown in Fig. 1.

Referring more specifically to the drawings, Fig. 1 shows by way of example for illustrative purposes, apparatus for forming a hydrogen positive ion beam and for utilizing this beam to form a mosaic target for electrons, the target being contained in an electron camera tube attached during the process to the tube wherein the ion beam is generated. The main tube 10 containing the target 14 is shown connected to the auxiliary tube 11 by means of a narrow neck 12 which is adapted to be cut and sealed off after the mosaic target in the main tube has been formed. The tube 10 comprises an evacuated container 13 enclosing the target 14 which is to have a mosaic surface formed thereon, an electron gun 15 suitable for generating and focussing a beam of electrons upon the target, and two sets of deflecting elements comprising the magnetic coils 16, 16 and 17, 17. The electron gun comprises, for example, a cathode 20, a cathode heater 21, a control electrode 22, a first anode 23, a second anode 24, and a conducting coating 25 which is preferably placed at the same potential as the second anode 24.

The target 14 is placed in position within the camera tube so that it can be struck by the electron beam generated and focussed by the gun 15, and also opposite an opening 26 in the conducting coating 25 through which radiations from an object are adapted to be applied to the target when the tube is finally completed and operating. During the formation of the mosaic surface on the target 14, however, the electron gun 15 is non-operative and radiations are not applied to the target. The target 14 preferably comprises a metallic backing plate 30 having a thin layer of mica or glass 31 held thereon by any suitable means, such as by screws or clamps (not shown). The insulating coating 34 has applied thereto by evaporation a thin layer 32 of a non-conducting me-

tallic oxide layer such as, for example, an oxide of one of the alkali or alkaline earth metals or an easily reducible non-conducting salt of one of these metals. One way in which a suitable non-conducting layer can be formed is by plating a coating of aluminum on the mica or glass layer 31 and then oxidizing this coating by any well-known means to form the layer 32. The layer 32 is then treated by means of the ion beam generated in the side tube 11 in a manner which will be described more fully below.

The tube 11, which is connected to the tube 13 by means of the neck 12 at a point thereof somewhere between the region of the gun 15 and the deflecting coils 16, 16 and 17, 17, comprises an evacuated container 40 enclosing a first electrode 41, a second electrode 42, and a third electrode 43. The electrode member 41 has been shown as a flat plate while the electrodes 42 and 43 have been shown as cylinders, the cylinder 43 being of larger diameter than the cylinder 42. The electrode member 41 is connected to the electrode 42 through a source 44 and two make-and-break contact members 45 and 46, the purpose of which will be described below. The positive pole of the source 44 is connected to the electrode member 41 and the negative pole thereof is connected through the members 45 and 46 to the electrode member 42. The electrode member 43 is placed at a negative potential with respect to the member 42 by means of a source 47 while the backing plate 30 of the target 14 in the tube 13 is placed at a negative potential with respect to the electrode member 43 by means of the source 48. A side tube 49 is connected to any suitable source of hydrogen.

The manner in which the apparatus shown in Fig. 1 operates to produce a positive ion hydrogen beam at the target 14 is as follows: The tube 11 is connected to the tube 10 by means of the glass neck 12. If it is desired to photosensitize the target while it is in the camera tube, the target cannot be exposed to the air without losing its photosensitivity. For this reason the electron gun 15 is mounted in the tube 10 and the conducting coating 25 is applied to a portion of the walls of the enclosure 13 by well-known means before the tube 11 is joined to the tube 10. Moreover, the target structure comprising the signal plate 30, the insulating layer of mica or glass 31, and the thin layer 32 of a non-conducting metallic oxide is placed in position before these two tubes 11 and 12 are joined together. A yoke holding the magnetic coils 16, 16 and 17, 17 is placed around the tube 10 (in some cases it may be desirable to perform this step also before the tube 10 is connected to the tube 11), and magnetic deflecting current is applied to these coils, which current may be of saw-toothed wave form or stepped wave form as will be described more fully below. No potentials are applied to the members of the electron gun 15 as the electron beam does not enter into the process of making the mosaic target coating. A magnetic coil schematically represented by the circle 50 is placed in position so that the beam of hydrogen positive ions when formed in the side tube 11 is directed toward the target 14. Hydrogen is admitted to the tube 11 from the side tube 49 and all other gases are removed from the tube 11 by means of the side tube 51, heat being applied during this step if necessary. Side tube 51 is sealed off after all occluded gases are removed from both of the tubes 11 and 13. With the electrode elements 41, 42

and 43 connected as shown in Fig. 1 of the drawing, the element 42 is at a negative potential with respect to the electrode member 41 inasmuch as the top half (as shown in Fig. 1) of each of the contact members 45 and 46 is of conducting material, while the bottom half of each is of non-conducting material. A stream of hydrogen positive ions is thus formed between the members 41 and 42. This stream is focussed into a beam by means of the electrostatic fields between members 42 and 43 which are at appropriate negative potentials with respect to the member 41 and thus "accelerate" the positive ions to produce a focussing action thereon in a manner similar to that produced on electrons by cylinders connected at positive potentials with respect to a cathode. This beam is focussed to a small cross-section at the surface of the target 14, the beam being bent by the constant current applied to the magnetic coil represented schematically by the circle 50. Source 48 can be omitted but in many cases it may be desirable to have an additional "accelerating" field between the electrode element 43 and the target 14. If saw-tooth current waves which are of uniform slope are applied to the coils 16, 16 and 17, 17, the frequency of these waves can be of the order, respectively, of the line scanning and frame scanning frequencies used in the usual television system. The members 45 and 46 are rotated at such speeds respectively that the member 46 makes contact for a period of time necessary to form an elemental particle 52 (see Fig. 2) and breaks contact (cutting off the beam) for a period of time corresponding to the distance between adjacent elemental particles 52. The member 45 is rotated at a somewhat slower speed and it acts to cut off the ion beam during alternate line scanning intervals so as to leave a space between lines as shown in Fig. 2. The frequency of rotation of the member 45 is equal to one-half the line scanning frequency of the wave applied to one of the coils 16, 16 or 17, 17, while the frequency of operation of the member 46 is equal to that of the member 45 divided by the number of elemental particles 52 it is desired to make in a line. If desired, the member 45 can be omitted and every line scanned, the beam being a little narrower than the line. Alternatively, the member 45 can be replaced by a corresponding member having a very narrow insulating segment to cut off the beam on the return trace between lines. Each particle 52 may be much less than an elemental area as determined by the size of the electron beam from the gun 15, or it may be substantially equal to the size of an elemental area and an adjacent insulating area or substantially as wide as an elemental area if the path of the electron beam is carefully controlled so that it goes over lines of sensitized metal islands and skips, by one means or another, the lines of insulation only. Each particle 52 is formed by reduction of the non-conducting metallic oxide by means of the hydrogen ions to produce a conducting metallic particle 52. In the presence of normal hydrogen the metal oxides are reduced extremely slowly, but under the impingement of ionized hydrogen the reduction is accelerated if at the same time the water vapor which is the decomposition product is pumped away thoroughly. The process therefore contemplates the circulation of very dry hydrogen at a low pressure through the tube during the reduction operation to remove the water vapor to keep it from recombining with the reduced metal. The hydro-

gen can enter through tube 49 and leave through tube 70, these two tubes being later sealed off. By means of the scanning method described above, each particle 52 is built up by successive 5 scannings of the ion beam over a surface of the insulating layers 31 containing the non-conducting oxide coating 32. At present it is believed that each particle 52 should be of the order of several hundred molecules thick and may take 10 many seconds or even several minutes before such a thickness is reached. If desired, the insulating spaces between particles 52 can be made less than or greater than the width of one of these particles. Preferably the insulating portions 15 should be as small as possible in order to provide as large an "active" area as possible.

In an alternative way of operating the arrangement shown in Fig. 1, stepped saw-toothed waves of line and frame scanning frequencies are applied to the coils 16, 16 and 17, 17. These waves are preferably of such low frequencies that one complete scanning of the target is sufficient to form by reduction each particle 52 of the desired density. By means of the stepped wave, the hydrogen ion beam is held stationary over an elemental area and remains on that elemental area until a sufficient amount of oxide is reduced to a conducting metal of the desired thickness on the target. Then the beam is almost instantaneously 20 jumped to the next elemental area leaving a space between the elemental areas blank as shown in Fig. 2. Such a stepped wave can be produced by a potentiometer having a number of taps with a rotating member connecting each of these taps 25 in turn to the magnetic coils. The potentiometers (one for the line and one for the frame scanning) can be geared together to maintain the two waves in proper time relation with each other or this may be done electrically as in ordinary television scanning. It will be clear that 30 the frequency of the wave applied to one set of coils 16, 16 and of that applied to the other set of coils 17, 17 have the same ratio as the two saw-toothed waves described above. When such current waves are used in the coils 16, 16 and 17, 17, the members 45 and 46 can be removed and replaced by a direct connection between the negative pole of the source 44 and the positive pole 35 of the source 47.

After the metal particles 52 are formed on the 40 insulating layer 31 by reducing portions of the oxide layer 32, the neck 12 is sealed off and the tube 10 evacuated and baked out so that all of the elements in the tube are thoroughly degassed. The tube is allowed to cool to room temperature 45 and oxygen is then admitted so as to oxidize a very thin layer of metallic particles. At the conclusion of the oxidation process, excess gas is removed by evacuation and a known amount of caesium is admitted into the bulb by flashing a "caesium pill." The pill is flashed in a side tube or in the tube 10 so that caesium vapor passes into the latter to photosensitize the metallic particles 52. A description of a suitable process of 50 photosensitizing with a "caesium pill" and the composition of such a pill may be found in British Patent 381,606 to George R. Stillwell and Charles H. Prescott, Jr., complete accepted October 10, 1932. The tube 10 is then baked at a 55 temperature of about 200 to 225° C. for varying periods of time to remove all gases. The operation of the mosaic screen in the cathode ray tube 10 is similar to that of the well-known iconoscope tube described in an article entitled "The iconoscope" by D. K. Zworykin in the January 1934

Proceedings of the Institute of Radio Engineers, pages 16 to 32, inclusive, and an article by the same author in the July 1936 "RCA Review," page 60, entitled "Iconoscopes and Kinescopes in Television."

An alternate way of forming the target is to use a plate of aluminum or a plate of other metal on which aluminum is plated, oxidize the aluminum to a predetermined depth, and then produce by the reduction process outlined above metal islands of a lesser depth than the oxide so that the oxide layer insulates under the islands as well as around them.

The tube 11, as mentioned above, can be used over and over again for the preparation of targets in storage type tubes, it being merely necessary to connect it to each tube in turn, go through the process described above and then break the connection between the tubes.

Fig. 3 shows apparatus of somewhat different form from that shown in Fig. 1 for utilizing a hydrogen positive ion beam to form a mosaic target for electrons. In the arrangement of Fig. 3, deflecting plates 60, 60 and 61, 61 are used to replace the magnetic coils 16, 16 and 17, 17 of Fig. 1 which are used to cause the hydrogen ion beam to scan the mosaic target 14. The magnetic bending field 50 is not required in the arrangement of Fig. 3 due to the fact that the tube 11 is joined to the tube 10 at such an angle that the axis of the hydrogen positive ion beam in its un-deflected position strikes the center of the target 14. Each of the elements of the apparatus which is common to the structures shown in Figs. 1 and 3 has been given the same reference character in both figures. The hydrogen positive ion beam is formed in the tube 11 in the manner described above in connection with Fig. 1 and the photo-sensitive mosaic is formed on the target 14 as described above with the exception that the scanning is caused by means of voltage waves applied to the deflecting plates 60, 60 and 61, 61 instead of current waves passed through the magnetic coils 16, 16 and 17, 17. After the tiny particles 52 are formed on the insulating layer 31, the neck 12 is broken and tube 10 is sealed up, evacuated and allowed to cool. The metallic particles 52 are then wholly or partially oxidized by any suitable method and photosensitized as in the process described above. The deflecting plates 60, 60 and 61, 61 are left within the tube 10. The process performed by the apparatus of Fig. 3, in some respects is preferable to that of Fig. 1 inasmuch as it is somewhat difficult to bend an ion beam by electromagnetic means due to the large mass of the ion as compared with that of the electron whereas electrostatic deflection may be obtained with field strength of the order of those commonly used to deflect an electron beam. Another advantage is simplification, the magnetic bending field 50 or an electrostatic equivalent thereof not being required.

As the metal of the particles 52 is such that it has to be photosensitized, the mosaic pattern can be applied in a separate tube or receptacle and then exposed to the air before being inserted in the cathode ray transmitter tube. The transmitter tube, in this modified arrangement, has means for admitting the sensitizing metallic vapor but has no positive ion gun associated with it at any stage of the process. In this arrangement the target is preferably placed at right angles to the beam.

Alternatively, a tube such as tube 11 of Fig. 3 can be connected to the tube 10 by means of a

rubber hose or similar connection 62. After the target has been provided with a metallic pattern by the reducing process described above, air can be admitted, the connection 62 broken and the opening sealed up. This alternative arrangement reduces the handling of the target after the formation of the pattern thereon. The tube 10 is then degassed, oxidized and sensitized in any known manner.

While the invention in its primary aspects relates to processes of or means for forming a mosaic target for use with an electron beam, it will be appreciated that the invention in its broader aspects is not limited to producing a target as the coating may be provided for some other purposes for which coatings are used. It will be understood also that various modifications can be made in the specific embodiments described above without departing from the principles upon which the invention is based.

What is claimed is:

1. The combination with a vessel, of means for producing a hydrogen atmosphere therein, spaced electrodes within said container between which said hydrogen is present, a source of potential having its terminals connected to said electrodes respectively whereby hydrogen positive ions move to one of said electrodes and electrons move to the other of said electrodes, an aperture in said electrode toward which said positive ions move and through which some of them pass, and a target for receiving said positive hydrogen ions, said target comprising an element of insulating material containing a coating of non-conducting metallic oxide and a conducting backing for said insulating material which backing is electrically connected to said apertured electrode.

2. The combination with a vessel, of means for producing a hydrogen atmosphere therein, spaced electrodes within said container between which said hydrogen is present, a source of potential having its terminals connected to said electrodes respectively whereby hydrogen positive ions move to one of said electrodes and electrons move to the other of said electrodes, an aperture in said electrode toward which said positive ions move and through which some of them pass, and a target for receiving said positive hydrogen ions, said target comprising portions of a material which can be reduced by hydrogen.

3. The combination with a vessel, of means for producing a hydrogen atmosphere therein, spaced electrodes within said container between which said hydrogen is present, a source of potential having its terminals connected to said electrodes respectively whereby hydrogen positive ions move to one of said electrodes and electrons move to the other of said electrodes, an aperture in said electrode toward which said positive ions move and through which some of them pass, a target for receiving said hydrogen positive ions, said target comprising an element of insulating material containing a coating of non-conducting metallic oxide and a conducting backing for said insulating material which backing is electrically connected to said apertured electrode, and means for causing said positive ion beam to scan said target, whereby said coating is produced in a progressive manner.

4. The combination with a vessel, of means for producing a hydrogen atmosphere therein, spaced electrodes within said container between which said hydrogen is present, a source of potential having its terminals connected to said electrodes respectively whereby hydrogen positive ions move

to one of said electrodes and electrons move to the other of said electrodes, an aperture in said electrode toward which said positive ions move and through which some of them pass, a target for receiving said positive hydrogen ions, said target comprising an element of insulating material containing a coating of non-conducting metallic oxide and a conducting backing for said insulating material which backing is electrically connected to said apertured electrode, and means including apparatus for causing said positive ion beam to impinge on discrete elemental areas of said target in succession to cause said coating to be produced by reduction in the form of discrete portions forming a regular pattern.

5. The method of metallic coating which comprises ionizing hydrogen in an electric field formed between two electrodes in an evacuated container, focussing the positive ions formed by said ionization into a beam which is highly concentrated and of relatively small cross-sectional area, and causing said beam to scan a two-dimensional portion of a target surface comprising an electrically non-conducting compound of one of the metals from the group consisting of the solid metals in group II in the periodic table and aluminum.

6. The method of making a mosaic target for an electron beam which comprises ionizing hydrogen in an electric field formed between two electrodes in an evacuated container, focussing the positive ions formed by said ionization into a beam which is highly concentrated and of relatively small cross-sectional area, and causing said beam to scan a two-dimensional pattern on a target surface comprising an electrically non-conducting compound of one of the metals from the group consisting of the solid metals of group II in the periodic table and aluminum to produce by reduction a uniform pattern of metallic and non-conducting portions, and photosensitizing the metallic portions of said pattern.

7. The method of making a mosaic target for an electron beam which comprises ionizing hydrogen in an electric field formed between two electrodes in an evacuated container, focussing the positive ions formed by said ionization into a beam which is highly concentrated and of relatively small cross-sectional area, and causing said beam to scan a two-dimensional pattern on a target surface comprising an electrically non-conducting oxide of one of the metals from the group consisting of the solid metals of group II in the periodic table and aluminum to produce by reduction a uniform pattern of metallic and non-conducting portions, and photosensitizing the metallic portions of said pattern.

8. The method of making a mosaic target for an electron beam which comprises ionizing hydrogen in an electric field formed between two electrodes in an evacuated container, focussing the positive ions formed by said ionization into a beam which is highly concentrated and of relatively small cross-sectional area, causing said beam to scan a two-dimensional pattern on a target surface comprising an electrically non-conducting oxide of one of the metals of the group consisting of the solid metals of group II in the periodic table and aluminum to produce by reduction a uniform metallic pattern, rapidly removing during the reduction the water vapor produced thereby, and after the pattern is pro-

duced photosensitizing the metallic portions of said pattern.

9. The method of metallic coating which comprises ionizing hydrogen in an electric field formed between two electrodes in an evacuated container, focussing the positive ions formed by said ionization into a beam which is highly concentrated and of relatively small cross-sectional area, causing said beam to scan a two-dimensional portion of a target surface comprising an electrically non-conducting oxide of one of the metals from the group consisting of the solid metals of group II in the periodic table and aluminum to produce by reduction a uniform pattern of metallic particles separated by non-conducting oxide particles, and circulating dry hydrogen during the reduction process to rapidly remove the water vapor produced during said process.
10. The method of metallic coating which comprises ionizing hydrogen in an electric field formed between two electrodes in an evacuated container, focussing the positive ions formed by said ionization into a beam which is highly concentrated and of relatively small cross-sectional area, and causing said beam to scan a two-dimensional portion of a target surface comprising an electrically non-conducting compound of one of the metals in the group consisting of the solid metals of group II in the periodic table and aluminum in a manner to produce a multiplicity of metallic islands, said islands being of less depth than the non-conducting compound whereby each island has some of the non-conducting compound under it as well as around it.
11. In the method of making a mosaic target for an electron beam, the combination of the steps of ionizing hydrogen in an electric field formed between two electrodes in an evacuated container, focussing the positive ions formed by said ionization into a beam which is highly concentrated and of relatively small cross-sectional area, and causing said beam to scan a two-dimensional portion of a target surface comprising an electrically non-conducting oxide of one of the metals from the group consisting of the solid metals of group II of the periodic table and aluminum in a manner to produce a multiplicity of metal islands.
12. In the method of making a mosaic target for an electron beam, the combination of the steps of plating a metal from the group consisting of the solid metals of group II of the periodic table and aluminum on another metal, oxidizing the metal plating to a predetermined depth, reducing selected portions of the oxide layer to such an extent that metal islands of less depth than the oxide layer are produced, whereby each island has oxide under it as well as around it, and photosensitizing the metal islands.

JOHN B. JOHNSON.

#### REFERENCES CITED

- 65 The following references are of record in the file of this patent:

#### UNITED STATES PATENTS

|    | Number    | Name                   | Date          |
|----|-----------|------------------------|---------------|
| 70 | 2,178,233 | Klatzow _____          | Oct. 31, 1939 |
|    | 2,239,642 | Burkhardt et al. _____ | Apr. 22, 1941 |
|    | 2,157,478 | Burkhardt et al. _____ | May 9, 1939   |